

Dec. 17, 1946.

G. G. PIERSON

2,412,693

METHOD AND TAPE FOR JOINING PLIES

Filed Jan. 26, 1940

*Fig. 1.*



*Fig. 2.*



*Fig. 3.*



*Fig. 4.*



*Inventor.*

Gordon G. Pierson

*by* *John G. Johnson and Son*  
*Attorneys.*

*Witness:*  
*Walter Chinn.*

## UNITED STATES PATENT OFFICE

2,412,693

## METHOD AND TAPE FOR JOINING PLIES

Gordon G. Pierson, Lansdale, Pa.

Application January 26, 1940, Serial No. 315,828

7 Claims. (Cl. 154—118)

1

This invention relates to improvements in methods of joining sheets of thin wood veneers that are adapted to be applied to a suitable material in the manufacture of panelling and other veneered products and of securing the sheets to a ply or base. The invention relates also to the products secured.

The present application is a continuation in part of my application for patent for Veneer tapes, filed April 18, 1938, Serial No. 202,809.

In the art of manufacturing plywood or veneers several sheets of thin wood are laminated by means of glue. The laminæ of wood for the aforesaid purpose may consist of whole sheets of wood or may be formed by abutting several smaller pieces and joining them at their edges in order to yield a large sheet. The essential joining has customarily been accomplished by gluing the edges of the sheets together with ordinary glue or, even more commonly, by gluing a narrow sheet of paper or a type of film known as a veneer tape which extends over the lateral surfaces of the veneer close to and overlapping the abutting edges of the veneer pieces.

In the past there have been several disadvantages to joining the sheets of wood with a paper or a film glued to their lateral surfaces over their contiguous edges. First, although the veneer tape or paper has held the pieces of wood together satisfactorily while they are being handled during the process of assembling the laminations, yet the bond in the finished lamination is extremely weak and insecure whenever the tape is used "within a glue line," that is, between a base and a veneer which is glued upon it.

A second disadvantage is that if tapes or films be sufficiently strong to permit easy handling of the larger sheets of veneer which have been thus assembled from separate veneer strips, then they are necessarily so thick that undesirable ridges appear on the surfaces of the finished laminations wherever the tape has been applied within the glue line.

A third difficulty arises because whenever ordinary veneer tapes are used inside of glue lines, the bond at that point has had an extremely low moisture resistance, regardless of the moisture-resistance properties of the glue used in making the lamination. In some types of laminations it has been possible to turn the veneer tapes i. e., to apply the tape to the opposite side of the veneer from that which faces the base, in order that the tapes may become exposed on the surface of the panel not within the glue lines. In such cases it becomes necessary to sand or to scrape the surface of the panel for the purpose of removing the tape before the panel can be finished. Obviously, drastic sanding or scraping is not only an expensive operation but may cut through the veneer and impair the panel.

2

The object of this invention is to eliminate broadly these usual undesirable features by making a veneer tape in a manner to be described subsequently.

5 A further object is to impregnate a tape with a glue suited to the glues used for uniting veneer to its base so that the bond between the one side of the tape and the veneer and also the bond between the tape and the base may be strengthened by the impregnation and made equally effective and the impregnation may protect the tape from weakening by moisture.

10 A further object is to strengthen and protect the tape by impregnation and not only to improve the tape surface for gluing purposes but to make the two sides equally effective for glue reception.

15 A further object is to form sturdier panels than before, which therefore may be subjected to vigorous handling during shipment and installation. 20 Accordingly, not only is undue waste of material avoided but considerable time is conserved in working with laminated sheets that are now less subject to injury by the mishaps and the exigencies of promiscuous handling.

25 A further object is to strengthen the hold of an adhesive by setting up a glue gradient tapering off from a full concentration outside the tape to a weaker glue in the middle of the tape thickness.

30 An additional object is to produce a moisture-resistant or moisture-proof panel whenever the veneer tape is used within the glue line.

35 For the purpose of illustrating the invention, the accompanying drawing illustrates several forms which are at present preferred, since the same have been found in practice to give satisfactory and reliable results, although it is to be understood that the several instrumentalities of the invention can be variously arranged and organized and that the invention is not limited to the precise arrangement and organization of the instrumentalities as herein shown and described.

40 The invention relates to several other novel features of construction and advantage appearing as hereinafter described and claimed in connection with the accompanying drawing in which:

45 Figure 1 is a broken perspective view of the invention showing two pieces of veneer partly joined by means of veneer tape.

50 Figure 2 is a section taken upon line 2—2 of Figure 1 in reverse position, i. e., with the tape on the under side ready for gluing to a base which is also shown.

55 Figure 3 is a section corresponding generally to Figure 2 but with the parts applied and with a base having a layer of veneer already applied and showing corresponding layers of veneer on the opposite face of the base.

60 Figure 4 is a section much like Figure 3 but

with a slightly different arrangement of the parts.

In the drawing similar numerals indicate like parts.

1 and 2, 1' and 2' represent pieces of veneer which abut at their edges, 1 against 2, and in another layer 1' against 2', and which form parts respectively of larger sheets, the several pieces being held together by veneer tape 3 engaging the surfaces at 4 and 5 on opposite sides of the line of veneer juncture 6. Meeting edges at 6 may be and in many cases are joined by glue.

The tape is used to hold the pieces together in order that the larger veneer sheets which are to be applied, may be handled as sheets. High effectiveness can best be secured and maintained with a tape which is as thin as practicable.

In the prior art veneer held together by tape normally was applied to the base such as 7 with the tape down as in Figures 2 and 3, bringing the tape "within the glue line" but in some instances it was applied to a base with the tape facing away from the base, as would be the case if the sheet of Figure 1 were applied as are the pieces 1' and 2' in Figure 4.

Where the tape is on the side of the veneer away from the glue line it is necessary to remove the tape by sanding or scraping unless another ply is to be added.

My invention is directed primarily to the use of the tape between two plies, whether between the veneer and the original base, or between two sheets of veneer. I have invented also a new tape.

The word base is used here generically without regard to whether the ply in question be a single ply only, as in Figure 2, or whether before the application of the veneer the initial base in question has received one or more layers or plies of veneer as in Figure 3.

In both of Figures 2 and 3 the position of the tape when the veneer has been applied is considered to be "within the glue line," not true with the position in Figure 1; and this is still true whether the tape be located so as to cover the joint between the adjacent veneer strips as in all of the figures, or for some reason be applied where there is no joint, but only a recognized possible weak spot 6'. It is also true that the tape is within the glue line where it has been carried on the "outside" of a first ply of veneer as at 3' in Figure 4 which is covered by a second or outer veneer ply, or is glued initially to the "inside" of a second veneer ply as in Figure 3.

The veneer tape 3 consists of a very thin sheet or film of a porous, permeable and flexible material which has been impregnated by a strong adhesive. Such an impregnating adhesive should have the characteristic of being tenacious not only to the veneer tape itself but to the glue that is subsequently employed to make the lamination i. e. to hold the veneer to the base. To distinguish, this will be called the laminating glue.

Preferably the veneer tape is very thin. Silk would be effective because very strong and sufficiently porous but is too expensive for normal use. The material used for veneer tape must be free from any prior surface treatment that would tend to prevent complete impregnation of the fibers throughout the thickness of the tape or film. This means that there must not be any appreciable amount of sizing in the paper as manufactured.

For impregnating the tape the adhesives which have been most satisfactory in tests made by me

have been "animal" glue and casein. Both of these are regarded in this description as nitrogenous glues of animal origin. For some purposes good fish glue—also regarded by me as coming within the genus of nitrogenous glue of animal origin—is satisfactory, but the poorer qualities of fish glue are not wholly satisfactory. Starch can be used but is not as good as animal glue.

10 It will be noted that with full impregnation of the tape both surfaces of the paper are alike and react equally to the adhesives used.

It is desirable that the adhesive used for impregnation be the same as but more dilute than the adhesive used to unite the tape to the veneer sheets. In this arrangement the impregnating and tape-applying adhesives unite to give a progressively variant concentration of adhesive from the impregnating strength present at the middle of the thickness of the tape and increasing in strength toward the surface of the tape. My tests have indicated that the best results are secured with what is known in the trade as animal glue, as distinguished from fish glue and casein. For convenience in grouping adhesives together for the purpose of claiming my invention and except as otherwise clearly indicated I give the term nitrogenous glue of animal kingdom origin a meaning broad enough to include fish glue and casein as well as animal glue.

30 The adhesive used for impregnation is desirably applied in a thin, aqueous, hot solution which is however substantially more concentrated than the adhesives used for sizing paper. The sheet from which strips of tape ultimately are to be cut is preferably unsized, uncalendered paper. It is thoroughly impregnated with the hot solution and the excess of the impregnating adhesive is squeezed out of the paper by passing the paper between pressure rolls. The squeezing between the rolls tends also to squeeze the remaining adhesive very thoroughly into and through the paper or other tape material.

40 The weakness of prior paper tapes which were affected by moisture lay primarily in the lack of complete impregnation with glue, permitting the weakness of the unimpregnated central plane of the tape to be emphasized by moisture taken up by the tape. Impregnation protects against this in two ways; both because the impregnated paper is stronger than the paper was before impregnation, and because the glue does not take up moisture as rapidly as would the paper if unprotected by the glue.

50 55 The impregnating glues are preferably nitrogenous glues; this term covering animal glue as known in the trade, fish glue and casein. All of these glues as well as starch glue hold well to the chief laminating glues, which are casein, starch glue and urea-formaldehyde.

Though my purpose is not primarily to moisture-proof, and the impregnating glues which I have described are not in themselves moisture-proofing glues, it is nevertheless true that where a formaldehyde-containing laminating glue is used, the formaldehyde from this laminating glue affects the impregnating glue and tends to moisture-proof it. Of the impregnating glues named, casein is very much more nearly moisture-resistant than animal glue.

65 70 75 In the preferred embodiment of the invention, the tape will be impregnated with animal glue (the product commercially known as such) of comparatively high dilution, subsequently coated with animal glue of higher concentration for join-

ing together veneer sheets of a single ply, and finally coated on the opposite side with any of the well-recognized laminating glues for uniting one ply with the adjoining ply.

It will be evident that the tape may be produced indifferently by impregnating a large sheet of paper, drying it, subsequently coating on one side with glue and drying it, then cutting it into strips to be moistened and applied hot or cold or by handling the individual strips separately, impregnating them and printing glue on them as they are being applied to the veneer at the edges, without any necessity for intermediate drying.

In accordance with the invention as previously specified the following examples obtained from actual practice are hereby submitted:

*Example 1.*—A thin sheet of unsized paper is dipped into a hot 10:1 solution of animal glue. The paper is then removed, the excess glue is squeezed out and the completely impregnated film is dried and cut into strips of suitable size. One side of the film may now receive a surface coat of a more concentrated solution of animal glue and this side may be applied to the veneer surfaces in the customary manner in order that a single sheet consisting of several pieces of veneer is in condition to be assembled with other sheets to form a lamination or a panel. To form the lamination, the single sheets composed of several pieces of joined veneer are coated, or the base material is, with the laminating glue and pressed in the conventional manner. Both may be coated.

The strength of the bond between the impregnated tape and the sheets of veneer in the finished lamination or plywood is as great as or greater than that between the untaped sheets of wood and is definitely much stronger than anything ever produced with veneer tapes heretofore employed.

I have made tests under like conditions to determine the sheer strength which have resulted as follows.

Average sheer values for three ply  $\frac{1}{8}$ " thick birch veneer expressed in pounds per square inch are as follows:

|                                                                            | Lbs. per sq. in. |
|----------------------------------------------------------------------------|------------------|
| Wood joined to wood by strong glue                                         | 400              |
| Wood covered with ordinary veneer tape and then joined with strong glue    | 100              |
| Wood covered with impregnated veneer tape and then joined with strong glue | 450              |

*Example 2.*—As has been previously mentioned, many kinds and combinations of strong glues may be used for impregnating the film or tape and for attaching it to a wood surface and for a subsequent gluing of the assembly in a lamination. As an example, casein glue may replace the animal glue of Example 1. The lamination may then be made with a starch glue in the conventional manner; or a urea resin glue, using either the cold or the hot pressing method, may replace the starch glue for the laminating process. When non-water resistant glues are used to impregnate or attach veneer tape to wood, and the lamination is then effected with a hot press resin glue containing formaldehyde, the entire assembly becomes water resistant because of the formaldehyde that is released from the resin by heat.

With laminating glue it is desirable to have as little water as possible and the proportion may well be about two parts of water to one of glue. On the other hand with impregnating glue the strengths which I have found desirable range from about five parts of water to one of glue to

sixteen parts of water to one of glue, the best results using about ten parts of water to one of glue. The preferable limit of dilution will be twelve to one. These were animal glues and the same proportions are correct for casein and good fish glues.

Not only is there an advantage in using the same adhesive for impregnation and subsequently for holding the tape to the sheets of veneer of a single ply, animal glue to animal glue, or casein to casein but the impregnated surface on the opposite side more readily receives the laminating glue. In a variant form of the invention, unsized and preferably also uncalendered paper is coated with a glue or nitrogenous glues of animal kingdom origin to glue together two veneer sheets to make a ply without prior impregnation and then a laminating glue as mentioned above is applied using such a high pressure as to force the laminating glue to impregnate the unsized paper. This procedure is not possible where conventional or sized paper is employed. The paper as in the other cases mentioned should be quite thin, of the order of one, two or three thousandths of an inch.

While the construction as shown and described is the preferred embodiment of the device, nevertheless the same may be modified in detail without departing from the spirit and the scope of the invention as defined in the annexed claims.

Having thus described my invention what I claim as new and desire to secure by Letters Patent is:

1. The method of joining veneer strips to a base by adhesives using a strip of unsized porous material, which consists in impregnating the strip, prior to assembling the veneer strips, with one concentration of nitrogenous adhesive of animal kingdom origin which becomes sticky when moistened to make a tape having the two faces of the tape alike, and cause each to present a surface which will readily bond with adhesive without rendering the body of the tape impervious to moisture, in gluing the tape to surfaces of the abutting veneer strips and across the joint in the veneer to hold strips of veneer together into a sheet using the same type of adhesive which becomes sticky when moistened but of greater concentration than that used for the impregnation and in then gluing the composite sheet of veneer thus formed to the base with the tape within the glue line by an adhesive containing moisture.

2. A woodworking veneer tape comprising an unsized paper strip impregnated with an adhesive which becomes sticky when moistened of a concentration of from about five to sixteen parts of water to one of adhesive and a ply of wood glued to one side of the paper strip by adhesive of the same character as the adhesive used in the impregnation and of greater concentration than that used in the impregnation.

3. The method of moisture-proofing the adhesive used for holding a tape to plies of veneer to be secured to a base which consists in impregnating tape of unsized paper with an adhesive prior to attachment to the veneer, uniting the tape to the veneer by the same kind of adhesive and gluing the taped veneer to the base by a glue which contains moisture and which liberates formaldehyde, whereby the moisture tends to remoisten the tape adhesives and the formaldehyde in due time tends to moisture-proof the adhesive in the tape and, through it, the adhesive holding the tape to the veneer.

4. The method of uniting plies of wood which

consists in gluing to veneer sheets making up a single ply, a tape of unsized paper freely permeable to glue and moisture from one side to the other, gluing together the plies under heavy pressure and impregnating the unsized paper by laminating glue containing moisture used between the plies due to the action of the pressure, the moisture of the laminating glue and the laminating glue being free to penetrate into the paper.

5. The method of joining veneer strips to a base by adhesives using a tape of moisture and glue permeable paper, which comprises coating the permeable paper of the tape with a cold setting tape-adhesive which becomes sticky when moist, without rendering the tape impervious to moisture, moistening the tape adhesive and while it is moist gluing the tape to surfaces of abutting veneer strips to hold the strips together into a sheet, still without rendering the tape impervious to moisture, and gluing the composite sheet of veneer thus formed to the base, under pressure, with the tape within the glue line, by a laminating adhesive containing moisture, whereby the moisture of the laminating adhesive is free to penetrate to and remoisten the tape adhesive while under the laminating pressure.

6. The method of joining veneer strips to a base by adhesives using a tape of moisture and glue permeable paper, which comprises coating and permeating the permeable paper of the tape with a cold setting tape adhesive which becomes sticky when moist, without rendering the tape

impervious to moisture, moistening the tape adhesive and while it is moist gluing the tape to surfaces of abutting veneer strips to hold the strips together into a sheet, still without rendering the tape impervious to moisture and gluing the composite sheet of veneer thus formed to the base, under pressure, with the tape within the glue line, by a laminating adhesive containing moisture, whereby the moisture of the laminating adhesive is free to penetrate to and remoisten the tape adhesive while under the laminating pressure.

7. The method of joining veneer strips to a base by adhesives, using a tape of moisture and glue permeable paper, which comprises coating the permeable paper of the tape with a cold setting tape adhesive which becomes sticky when moist, without rendering the tape impervious to moisture, moistening the tape adhesive and while it is moist gluing the tape to surfaces of abutting veneer strips to hold the strips together into a sheet, still without rendering the tape impervious to moisture, and gluing the composite sheet of veneer thus formed to the base under pressure, with the tape within the glue line, by a laminating adhesive containing moisture and liberating formaldehyde, whereby the moisture of the laminating adhesive is free to penetrate to and remoisten the tape adhesive while under the laminating pressure and the formaldehyde in due time tends to make the assembly moisture resistant.

GORDON G. PIERSON.